

J. H. BECKER.  
METHOD OF MAKING SPARK PLUGS.  
APPLICATION FILED JUNE 11, 1919.

1,331,091.

Patented Feb. 17, 1920.



John H. Becker, Inventor  
By his Attorney,  
W. B. Hutchinson,

# UNITED STATES PATENT OFFICE.

JOHN H. BECKER, OF NUTLEY, NEW JERSEY.

## METHOD OF MAKING SPARK-PLUGS.

1,331,091.

Specification of Letters Patent. Patented Feb. 17. 1920.

Application filed June 11, 1919. Serial No. 303,372.

*To all whom it may concern:*

Be it known that I, JOHN H. BECKER, a citizen of the United States, and a resident of Nutley, Essex county, New Jersey, have 5 invented a new and useful Improvement in Methods of Making Spark-Plugs, of which the following is a full, clear, and exact description.

My invention relates to improvements in 10 the method of making spark plugs, and more particularly in the method of securing the core or porcelain in the outer or metallic shell. Owing to the different co-expansions 15 of spark plug cores and their shells, there is a good deal of difficulty in making a perfectly tight union between the parts especially where attempts to do this are made without using gaskets, nuts, or the like. These extraneous fastenings are objectionable 20 because in actual use when the plug becomes highly heated it often happens that the core breaks because of the stress upon it between its fastening devices, and where the core is fastened by simply shrinking the 25 metal upon it the loss by breakage is very great during the manufacturing operation. It is generally recognized that it is desirable 30 to have the core secured in its shell without any extraneous fastenings, but simply by having the shell shrunk upon the core. My invention provides a means for doing this so 35 that the loss during manufacture is negligible, and therefore my method is such that after the plug is made it is not liable to break, because the core is subjected to more strain during the process of manufacture than it ever is in actual use. My method, 40 therefore, is intended to provide a simple and efficient means of securing the core in the shell so that it will stand up under use, and so that a perfect union between the two parts will be had.

Reference is to be had to the accompanying drawing forming a part of this specification, in which similar reference characters 45 indicate corresponding parts in the view.

The drawing is a vertical section of a spark plug shell and core.

The shell 10 can be of any approved construction but it should have a slightly tapering section 11, and the core 12 can likewise be of any usual or preferred construction, except that it should have a section 13 shaped to fit tight against the corresponding part 11 of the shell. In my early attempts to shrink a shell of this character

upon a somewhat similar core, I found that the breakage of the core ran as high as 95%; but by carrying out my method as I have evolved it by repeated experiments, the 60 breakage is practically nothing, and the union between the shell and core is perfect so that no other fastening means is necessary. To accomplish this result I practically anneal the core, that is to say, I expel 65 all the moisture practicable, and toughen it by subjecting it for a comparatively long time to a heating but relatively low temperature. I have got the best results baking the core in an oven for about fifty hours at 70 a temperature of about 150 degrees F. The heating process may be made longer or shorter, but the time given gives the best results. Likewise the temperature can be varied somewhat, but should not be varied 75 much from the temperature given. In any event the temperature should not be less than 140 degrees or more than 170 degrees.

After the core has been toughened by the long preliminary treatment as specified, and 80 it is to be united permanently to the shell, the latter is heated to a cherry red heat, that is to say, to a temperature of approximately 1400 degrees F., and this temperature should not be varied so as to be less than 1200 degrees or more than 1600 degrees, and the temperature given is preferable to either. The core is heated to the same temperature as the hot shell, and is then pressed into the shell so that the part 13 will seat itself 85 firmly in the part 11 of the shell, and then the shell is permitted to shrink by cooling so as to become absolutely fixed upon the core.

If this method is carried out as stated 95 there will be comparatively no loss of cores by breakage, and the two parts will be so firmly united that they will never separate under use, and moreover, the joint will be so tight that there will be no leakage of gas or 100 current.

I claim:

1. The herein described method of securing spark plug cores in their shells, which consists in first toughening the core by subjecting it for a comparatively long time to a low temperature, then heating the shell and core to approximately the same temperature, and finally while both shell and core are hot, pressing the core into its seat in the 110 shell.

2. The herein described method of secur-

ing spark plug cores in their shells, which consists in first toughening the core by a long preliminary heating at a relatively low temperature, then heating the core and shell 5 to a high temperature, and finally pressing the hot core to its seat in the hot shell.

3. The herein described method of securing spark plug shells and cores, which consists in first toughening the core by heating 10 it for a long period to a temperature of not less than 140 degrees F. nor more than 170 degrees, next heating the shell and core to a high temperature, and finally pressing the hot core into the hot shell.

15 4. The herein described method of securing spark plug cores and shells, which consists in first toughening the core by a long pre-heating at a low temperature, next heating both core and shell to a temperature of

not less than 1200 degrees nor more than 20 1600 degrees F., then pressing the hot core to its seat in the hot shell, and finally cooling the united parts so that the shell shrinks upon the core.

5. A herein described method of uniting 25 spark plug shells and cores, which consists in providing the shell with a tapering seat, providing the core with a tapering portion to fit the seat, heating the core for a long period at a low temperature, then heating 30 the core and shell to a high temperature, and finally pressing the hot core to its seat in the hot shell.

JOHN H. BECKER.

Witnesses:

WARREN B. HUTCHINSON,  
M. G. O'DONNELL.